

N. E. SHERWOOD,

ROPE.

APPLICATION FILED JUNE 13, 1919.

1,331,679.

Patented Feb. 24, 1920.



Fig. 1.



Fig. 3.



Fig. 4.



Fig. 2.



Fig. 5.



Fig. 6.



Fig. 7.

Inventor

Nathan E. Sherwood,

By *Pagden & Spamer* Attorneys

# UNITED STATES PATENT OFFICE

NATHAN E. SHERWOOD, OF HIGHLAND PARK, MICHIGAN.

## ROPE.

1,331,679.

Specification of Letters Patent. Patented Feb. 24, 1920.

Application filed June 13, 1919. Serial No. 304,054.

*To all whom it may concern:*

Be it known that I, NATHAN E. SHERWOOD, a citizen of the United States, and residing at Highland Park, in the county 5 of Wayne and State of Michigan, have invented a new and Improved Rope, of which the following is a specification.

The object of the present invention is to provide a composite fiber and wire rope of 10 greater strength for a given size and weight than has been obtainable heretofore, and it consists in a rope formed from a plurality of strands of twisted hemp, sisal or other strong fiber said strands being simultaneously 15 tightly twisted together with one or more small wires of steel or other ductile metal having high tensile strength.

In the drawings, Figure 1 is a side view of a short section of the finished rope, 20 the ends being unraveled. Fig. 2 is a diagrammatic side view showing the several strands and wires that make up a single cord. Fig. 3 is a side view showing the preferred relation of the strands to one another 25 before twisting. Fig. 4 is a similar view after the parts have been twisted. Figs. 5, 6 and 7 are sections on the lines 5-5, 6-6 and 7-7 of Fig. 4.

It has been proposed to make sewing cord 30 of a plurality of strands each of which is formed of a plurality of fibres around which a wire is twisted—see U. S. patent to Briggs, 346,577, August 3, 1886. In practice, the wire thus placed forms a sheath for the corresponding strand, rather than a component 35 part thereof, and tends to unwind when tension is applied.

According to the present invention, I take a plurality of strands 1, Fig. 2, of usual 40 rope material (such as hemp or sisal "binder twine")- each of which comprises a number of fibers twisted together, and twist said strands tightly together with one or more wires 2 of iron or steel or other metal having 45 a high tensile strength, whereupon they assume the appearance indicated in Fig. 4. This action is to be carefully distinguished from what would occur were the several strands 1 first twisted together and there- 50 after wrapped or twisted around with a wire, even though the latter were of the same

pitch as the strands. In this latter case, the wire would always be on the outside of the strand, whereas, according to my invention, it is at certain points on the outside, again at 55 the center, and at still other points is intermediate between the two, as indicated in Figs. 4, 5, 6 and 7. The course of the wire is like that of any particular fiber of ordinary binder twine; and the practical result 60 is that the wire enters with the strands to form a cord or rope wherein both the tensile strength of the fiber and the tensile strength of the metal is efficiently utilized, and in which the fiber acts as a cushion for the wire, 65 thereby preventing breaking under sudden jerks.

The resulting small cord or rope is preferably finally twisted with additional cords or ropes as indicated in Fig. 1 thereby forming 70 a completed rope of a size sufficient to meet the particular need. For some purposes the single element shown in Fig. 4 will suffice. The number of strands 1 may, of course, be varied as may the number of 75 wires which go to make up the corresponding cord, but it is preferred to use four strands and two wires for each cord.

### I claim:

1. A cord formed of a series of strands of 80 twisted fiber such as hemp or sisal twisted tightly together and simultaneously with a wire of strong tensile metal twisted in with the strands of fiber so as to lie parallel therewith, whereby the position of the wire in the 85 cord is at some points on the outer surface of the cord and at other points is intermediate between the center of the cord and said outer surface.

2. A rope comprising a plurality of cords 90 tightly twisted together, each cord including a plurality of strands of twisted fiber and one or more small wires of strong tensile metal, twisted in with the strands of fiber so as to lie parallel therewith, said strands 95 and wire or wires being simultaneously twisted together, and the wire or wires being on the outer surface of the corresponding cord at some points and being near the center thereof at other points.

NATHAN E. SHERWOOD.